# EUROPEAN PATENT APPLICATION

(11) **EP 3 297 107 A1**
(43) Date of publication of application: **21.03.2018**
(21) Application number: 17196183.2
(22) Date of filing: 09.12.2015
(51) Int. Cl.: H01T 13/39, H01T 21/02

(54) **SPARK PLUG WITH CERAMIC ELECTRODE TIP**

(30) Priority: 19.12.2014 US 201414577174
(62) Divisional of application: 15198613.0
(71) Applicant: Federal-Mogul Ignition Company, Southfield, MI 48034 (US)
(72) Inventor: WALKER JR., Mr. William J., Toledo, OH 43606 (US)
(74) Representative: De Bonis, Paolo

(57) **Abstract**

A spark plug **(20)** for igniting a mixture of fuel and air of an internal combustion engine comprises a center electrode **(22)** and a ground electrode **(24).** At least one of the electrodes **(22, 24)** includes a body portion **(28, 30)** formed of thermally conductive material and a firing tip **(32, 34)** disposed on the body portion **(28, 30).** The firing tip **(32, 34)** includes a ceramic material, providing an exposed firing surface **(36, 38).** The ceramic material is an electrically conductive, monolithic ceramic material. The ceramic material of the firing tip **(32, 34)** includes at least one perovskite structure and/or at least one a spinel structure.

## Description

### CROSS REFERENCE TO RELATED APPLICATIONS

This application claims priority to U.S. Patent Application No. 14/577,174.

### BACKGROUND OF THE INVENTION

### 1. Field of the Invention

The invention relates generally to ignition devices for internal combustion engines, such as spark plugs, and more particularly to the electrodes therefore.

### 2. Related Art

Internal combustion engines include ignition devices, such as spark ignition devices or spark plugs that extend to the combustion chamber and produce a spark to ignite a mixture of air and fuel. Recent advancements in engine technology are resulting in higher engine operating temperatures to achieve improved engine efficiency. These higher operating temperatures, however, are pushing electrodes of the spark plugs to the very limits of their material capabilities. Presently, Ni-based alloys, including nickel-chromium-iron alloys specified under UNS N06600, such as those sold under the trade names Inconel 600®, Nicrofer 7615®, and Ferrochronin 600®, are typically used as spark plug electrode materials.

As is well known, the resistance to high temperature oxidation of these Ni-based nickel-chromium-iron alloys decreases as their operating temperature increases. Since combustion environments are highly oxidizing, corrosive wear including deformation and fracture caused by high temperature oxidation and sulfidation can result and is particularly exacerbated at the highest operating temperatures. At the upper limits of operating temperature (e.g., 1400°F), tensile, creep rupture and fatigue strength also have been observed to decrease significantly which can result in deformation, cracking and fracture of the electrodes. Depending on the electrode design, specific operating conditions and other factors, these high temperature phenomena may contribute individually and collectively to undesirable corrosion and erosion of the electrode and diminished performance of the ignition device and associated engine, especially in high performance engines, such as those used in automobile racing.

High temperature firing tips have been employed in conjunction with the electrode materials described. These firing tips have been manufactured from a number of platinum group metals and metal alloys, such as platinum, iridium, rhodium, palladium, ruthenium and rhenium, as pure metals and together with themselves and various other alloy constituents, such as various rare earth elements, in various alloy combinations; gold and gold alloys; tungsten and tungsten alloys and the like. These high temperature firing tips have been attached to a body portion of the electrode materials described above, both center and ground electrodes, in various tip configurations using a wide variety of attachment and joining techniques, including resistance welding, laser welding, mechanical joining and the like, both separately and in various combinations.

Notwithstanding the electrode performance improvements attainable through the use of high temperature firing tips, there remain various aspects of these materials which limit their application and use in ignition device configurations and applications, for example susceptibility to other and new high temperature oxidation, erosion and corrosion mechanisms, such as those associated with small amounts of calcium and phosphorus, thermal expansion mismatch with various center and ground electrode materials and other aspects, such as the high cost of these materials, which serve to limit their usefulness in various ignition applications.

### SUMMARY OF THE INVENTION

One aspect of the invention provides a spark plug for igniting a mixture of fuel and air of an internal combustion engine in accordance with Claim 1. Another aspect provides for a spark plug for igniting a mixture of fuel and air of an internal combustion engine according to Claim 8.

Another aspect of the invention provides a method of manufacturing a spark plug for igniting a mixture of fuel and air of an internal combustion engine in accordance with claim 15.

Yet another aspect of the invention provides an electrode for an ignition device according to Claim 14. The electrode comprises a body portion including a thermally conductive material, and a firing tip disposed on the body portion, wherein the firing tip includes a ceramic material. The ceramic material includes at least one perovskite structure and/or at least one spinel structure.

Another aspect of the invention provides a method of manufacturing an electrode for an ignition device. The method comprises compacting a ceramic material to form a firing tip, wherein the ceramic material includes at least one of a perovskite structure, a spinel structure, and a precursor material that forms a perovskite or spinel structure upon sintering. The method further comprises sintering the compacted ceramic material; and disposing the sintered ceramic material on a body portion including a thermally conductive material.

The electrode comprising the firing tip formed of the at least one perovskite structure and/or at least one spinel structure is economical to manufacture and provides a longer useful life, compared to other electrodes used in ignition devices. The combination of the thermally conductive body portion and ceramic firing tip provides resistance to high temperature oxidation, sulfidation, and related corrosion and erosion, while also effectively conducting heat from the firing tip to reduce the operating temperature at the firing tip.

### BRIEF DESCRIPTION OF THE DRAWINGS

Other advantages of the present invention will be readily appreciated, as the same becomes better understood by reference to the following detailed description when considered in connection with the accompanying drawings wherein:
Figure 1 is a cross-sectional view of a spark plug constructed in accordance with one embodiment of the invention;
Figure 1A is an enlarged cross-sectional view of the firing tips of the electrodes of Figure 1; and
Figures 2-11 are cross-sectional views of center electrodes according to other embodiments of the invention, including various different firing tip configurations.

### DETAILED DESCRIPTION

One aspect of the invention provides a spark plug 20 for igniting a mixture of fuel and air of an internal combustion engine. As shown in Figures 1 and 1A, the spark plug **20** includes a center electrode **22** and a ground electrode **24** providing a spark gap **26** therebetween. At least one of the electrodes **22, 24** includes a body portion **28, 30** formed of a thermally conducive material and a firing tip **32, 34** formed of a ceramic material disposed on the body portion **28, 30.** The ceramic material of the firing tip **32, 34** provides a firing surface **36, 38** for emitting a spark to ignite the mixture of fuel and air.

By forming the firing tip **32, 34** of the ceramic material, a lower operating temperature is provided at the firing tip **32, 34.** By forming the body portion **28, 30** of a thermally conductive material, heat is effectively conducted away from the ceramic firing tip **32, 34.** Thus, the electrode **22, 24** of the present invention, with the thermally conductive body portion **28, 30** and the ceramic firing tip **32, 34,** provides a lower operating temperature at the firing tip **32, 34** than other electrodes formed entirely of the ceramic material. The reduced operating temperature at the firing tip **32, 34** extends the life of the spark plug **20.** Further, the electrode **22, 24** of the present invention is more economical to manufacture than those with platinum group metal firing tips.

While the electrode **22, 24** is described for use in the particular spark plug **20** application of Figure 1, it will be appreciated that the electrode **22, 24** having the thermally conductive body portion **28, 30** and the ceramic firing tip **32, 34** can be used in other types of ignition devices.

As shown in Figure 1, the center electrode 22 extends longitudinally along a center axis **A** from a center electrode top end **40** to a center firing end **42.** The body portion **28, 30** of the center electrode **22**, referred to as a center body portion **28**, extends from the center electrode top end **40** toward the center firing end **42.** The center body portion **28** includes a thermally conductive material and is typically formed entirely of the thermal conductive material, but may be formed of multiple different thermally conductive materials. The center body portion **28** has a thermal conductivity sufficient to draw heat away from a center firing tip **32.** In one embodiment, the center body portion **28** has a thermal conductivity of at least 20 Wm-K when measured at 20° C, and preferably at least 35 W/m-K when measured at 20° C. The thermally conductive material of the center body portion **28** is also electrically conductive. The center body portion **28** also typically has an electrically conductivity of at least 9 x 10⁵ siemens per meter (S/m). The thermally conductive material is typical metal, preferably nickel or nickel alloy, or a mixture of different metals.

The center electrode **22** can include a variety of different configurations, as shown in Figures 2-11. In one embodiment, as shown in Figures 10 and 11, the center body portion **28** includes a clad **44** of a first thermally conductive material, such as nickel, and a core **46** of a second thermally conductive material, such as copper, enrobed by the clad **44.** The thermally conductive material of the core **46** is also electrically conductive.

As shown in Figure 2, the center body portion **28** has a first diameter **D₁** extending perpendicular to the longitudinal center body portion **28.** The first diameter **D₁** of the center body portion **28** is typically 2.69 mm, 2.16 mm, 1.83 mm, or 1.32 mm. However, it will be understood by those of ordinary skill in the art that the center body portion **28** may have other dimensions. In one embodiment, as shown in Figures 2-6 and 9-11, the center body portion **28** presents a center hole **48** extending longitudinally along the center axis **A** and facing outwardly of the center electrode **22** at the center firing end **42.** In the embodiment of Figure 10, the center hole **48** and the center firing tip **32** are spaced from the core **46** of the center body portion **28** by the clad **44.** In the embodiment of Figure 11, the center hole **48** and the center firing tip **32** abut the core **46.** In another embodiment, shown in Figures 3-10, the center electrode **22** has a diameter reduction, referred to as a third diameter **D₃**, along the center body portion **28** in a region spaced from the center firing end **42.** In yet another embodiment, as shown in Figures 4 and 9, the center electrode **22** has the reduced third diameter **D₃** along the center body portion **28** in the region spaced from the center firing end **42**, and tapers from the center body portion **28** to the center firing end **42** forming a frustum of a cone along a segment of the center body portion **28** adjacent to the center firing end **42.** In one embodiment, the third diameter **D₃** of the center electrode **22** is 2.54 mm, 1.98 mm, 1.65 mm, or 1.16 mm, corresponding to the first diameters **D₁** examples provided above. However, it will be understood by those of ordinary skill in the art that the center electrode **22** may have other dimensions. The center firing tip **32** also has a cylindrical geometry, but can comprise other shapes.

At least one of the electrodes **22, 24**, but preferably both electrodes **22, 24** include the ceramic firing tip **32, 34.** As shown in Figures 1-11, the center electrode **22** includes the firing tip **32**, referred to as the center firing tip **32**, formed of the ceramic material to provide a long-life center firing surface **36** for the spark plug **20.** The center firing tip **32** extends transversely from the center firing end **42.** The ceramic material of the center firing tip **32** presents the firing surface **36**, referred to as a center firing surface **36**, which is typically planar and faces outwardly for emitting a spark to ignite the mixture of fuel and air. In another embodiment, the center firing surface **36** is convex (not shown). In one embodiment, as shown in Figures 2-6 and 9-11, the center firing tip **32** is disposed in the center hole **48.** The center firing tip **32** typically has a second diameter **D₂** extending perpendicular to the center axis that is less than the first diameter **D₁** of the center body portion **28.** The second diameter **D₂** of the center firing tip **32** is typically 1.5 mm, 1.0 mm, or 0.7 mm. However, it will be understood by those of ordinary skill in the art that center firing tip **32** may have other dimensions. The center firing tip **32** also has a cylindrical geometry, but can comprise other shapes.

In one embodiment, the center firing tip **32** comprises a monolithic ceramic rivet, as shown in Figures 6-8. In yet another embodiment, as shown in Figure 8, the firing tip **32, 34** includes a first section and a second section, wherein the first section is disposed on the body portion **28, 30** and includes a metal material, and the second section is disposed on the first section and includes the ceramic material.

The center firing tip **32** includes a ceramic material presenting the center firing surface **36**, preferably a monolithic and electrically conductive or semi-conductive ceramic material. Typically, the center firing tip **32** is formed entirely of the electronically conductive ceramic material. In one embodiment, the ceramic material of the center firing tip 32 has an electrical conductivity of at least 10⁶ S/m. The appropriate ceramic material is used in the construction of the center firing tip **32**, depending on the level of resistance desired and the temperatures to which the center electrode **22** is exposed. Further, the ceramic material can be provided as a homogeneous material over the entire structure of the center firing tip **32**, or as a gradient or a composite. In one preferred embodiment, the ceramic material includes at least one of one of Titanium Diboride; Silicon Carbide; and Ternary Silicides, Nitrides and Carbides, such as Molybdenum Silicide Carbide (Mo₅Si₃C) or Titanium Carbonitride (TiCN), for example. Other examples of ceramic materials that can be used to form the center firing tip **32** are disclosed in U.S. Patent Application Nos. 12/200,244; 12/201,567; and 12/201,590, each to the present inventor, William J. Walker, Jr.

In one embodiment, the center firing tip **32** is formed of a ceramic material disclosed in U.S. Patent Application No. 12/200,244. The center firing tip **32** of this embodiment is preferably constructed entirely of a solid, one-piece, monolithic conductive or semi-conductive ceramic material. The ceramic materials can include, by way of example and without limitation, oxides, borides, nitrides, carbides, and silicides.

In one embodiment, the center firing tip **32** of the center electrode **22** is constructed of at least one oxide. For example, 100 weight percent (wt. %) of the center firing tip **32** could consist of the at least one oxide. Alternatively, at least 50 wt. %, or at least 70 wt. %, or at least 90 wt. %, or at least 95 wt. % of the center firing tip **32** could consist of the at least one oxide. The at least one oxide used to form the center firing tip **32** typically includes oxides of transition metals. In this embodiment, the oxides can include monoxides, such as TiO, VO, NbO, TaO, MnO, FeO, CoO, NiO, CuO, and ZnO; sesquioxides, such as V₂O₃, CrO₃, Fe₂O₃, RhO₃, In₂O₃, Th₂O₃, and Ga₂O₃; and dioxides such as TiO₂, VO₂, CrO₂, MoO₂, WO₂, RuO₂, ReO₂, OsO₂, RhO₂, IrO₂, PbO₂, NbO₂, MbO₂, MnO₂, PtO₂, GeO₂, and SnO₂.

In an exemplary embodiment, the at least one oxide of the center firing tip **32** comprises at least one perovskite structure, which is an oxide of two or more metals including at least one transition metal. The perovskite structures can have the general formulation ABO₃, wherein component A includes at least one of La, Ca, Ba, Sr, Y, and Gd; and component B includes at least one of Sc, Ti, Zr, Hf, Nb, Ta, Mo, W, Re, V, Cr, Mn, Tc, Fe, Ru, Co, Rh, Ga, and Ni. Examples of such perovskite structures include LaCrO₃, LaMnO₃, LaFeO₃, LaGaO₃, and LaCoO₃.

In another embodiment, at least a portion of the component A and/or at least a portion of the component B of the perovskite structure can be replaced or substituted with a another component C and/or component D. In other words, some of component A, or all of component A, could be replaced with component C and/or component D; and some of component B, or all of component B, could be replaced with component C and/or component D. In an exemplary embodiment, component C includes at least one of La, Ca, Ba, Sr, Y, and Gd; and is different from component A and B. Component D includes at least one of Sc, Ti, Zr, Hf, Nb, Ta, Mo, W, Re, V, Cr, Mn, Tc, Fe, Ru, Co, Rh, and Ni; and is different from component A and B. For example, the perovskite structure with the formulation ABO₃ could be substituted with the additional component C and/or component D to form a perovskite with the general formulation (AₓC₁₋ₓ)BO₃, A(B_{y}D_{1-y})O₃ or (AₓB₁₋ₓ)(C_{y}D_{1-y})O₃, wherein x is between 0 and 0.5 and y is between 0 and 0.5. A specific example of the alternate perovskite structure is La₁₋ₓSrₓMnO₃. wherein a portion of the La is substituted with Sr. In addition, in certain embodiments, there could be three or more elements that occupy component A, which are each selected from the list of component A above; and/or three or more elements that occupy component B, which are each selected from the list of component B above.

Furthermore, components C and D may include elements selected from a group that have a valence charge different from that of components A and/or B, so that the total amount of oxygen (O) can be greater than or less than 3. For example, the alternate perovskite structure could have the general formulation MₓN_{1-y}O_{3-z}, wherein component M comprises component A and at least one other metallic element; component N comprises component B and at least one other metallic element; x is in the range from 0.9 to 1.1; y is in the range from 0.9 to 1.1; and z is in the range from -0.2 to 0.2. In an exemplary embodiment, the at least one other metallic element of component M and/or component N is selected from the following group: La, Ca, Ba, Sr, Y, Gd, Sc, Ti, Zr, Hf, Nb, Ta, Mo, W, Re, V, Cr, Mn, Tc, Fe, Ru, Co, Rh, Ni, Cu, Zn, Ag, Ga, Al, and Si. In this embodiment, the valence charge of the other metallic element of component M is different than the valence charge of component A, and the valence charge of the other metallic element of component N is different from the valence charge of component B.

In another embodiment, the at least one oxide used to construct the center firing tip **32** of the center electrode **22** comprises at least one spinel structure, instead of or in addition to the at least one perovskite structure. The spinel structure can have the general formulation AB₂O₄, wherein component A includes at least one of Li, Co, Mg, Zn, Ni, Fe, Cd, Mn, and Cu; and component B includes at least one of Al, Cr, and Fe. An exemplary spinel structure is nickel ferrite, which is an electrically conducting spinel having the stoichiometric composition NiFe₂O₄. In one embodiment, the performance of the spinel is improved by changing the ratio of Ni and Fe, such that the general formulation of the spinel is Ni₁₋ₓFe₂₊ₓO₄ or Ni₁₊ₓFe₂₋ₓO₄, wherein x ranges from 0 to 0.5

In another embodiment, at least a portion of the component A and/or at least a portion of the component B of the spinel structure can be replaced with another component C and/or component D. In other words, some of component A, or all of component A, could be replaced with component C and/or component D; and some or component B, or all of component B, could be replaced with component C and/or component D. In an exemplary embodiment, component C includes at least one of Li, Co, Mg, Zn, Ni, Fe, Cd, Mn, Cu, Mo, W, Cr and V; and component C is different from component A and B. Component D includes at least one of Al, Cr, Fe, Co, Ga and Mo; and component D is different from component A and B. Like the perovskite structures, the spinels can be substituted, in which case the general formulation would be MₓN_{2-y}O_{4-z}, wherein M comprises component A and at least one other metallic element; N comprises component B and at least one other metallic element; x ranges from -0.1 to 0.1; y ranges from -0.1 to 0.1; and z ranges from -0.2 to 0.2. In an exemplary embodiment, the at least one other metallic element of component M and/or component N is selected from the following group: Ge, V, Te, Ti, Sb, Nb, Ta, W, Sn, Hf, Zr, Sc, Bi, and In.

The center firing tip **32** constructed of the perovskite structure or spinel structure is manufactured by compacting and sintering the ceramic material. In one embodiment, the ceramic material initially provided for compacting and sintering includes at least one of the perovskite structures or spinel structures described above.

In another embodiment, a precursor material is provided which upon sintering forms one of the perovskite structures or spinel structures. The precursor material typically includes common oxides and/or carbonates of the elements listed above. Exemplary precursor materials that can be compacted and sintered to form the center firing tip **32** from a perovskite structure include at least one of La₂O₃, CaCO₃, BaCO₃, SrCO₃, Y₂O₃, Gd₂O₃, Sc₂O₃, TiO₂, ZrO₂, HfO₂, Nb₂O₅, Ta₂O₅, MoO₃, Mo₂O₃, WO₃, ReO₃, V₂O₃, Cr₂O₃, MnO₂, Fe₂O₃, FeO, Fe₃O₄, RuO₄, CoO, NiO, and Ni₂O₃. Exemplary precursor materials that can be compacted and sintered to form the center firing tip **32** from a spinel structure include at least one of Li₂CO₃, CoO, MgCO₃, MgO, ZnO, NiO, Ni₂O₃, FeO, Fe₂O₃, Fe₃O₄, CdO, MnO₂, CuO, Al₂O₃, Al(OH)₃ and Cr₂O₃.

The borides include, for example, chemical compositions having the formula MₓB_{y}, where M is a metallic element, X is often 1, and Y is often 1, 2 or 6. Other examples include borides having an electrical resistivity in the range of 10⁻⁵ to 10⁻⁴ ohm-cm, and melting points in the range of 1600 to 3200 degrees Celcius. Specific examples include Zirconium Boride (ZrB₂; ZrB and ZrB₁₂); Hafnium Boride (HfB₂); Titanium Boride (TiB₂; TiB); Vanadium Boride (VB₂; VB); Tungsten Boride (W₂B₅); Chromium Boride (CrB₂; CrB); Molybdenum Boride beta-MoB, alpha-MoB, Mo₂B₅; Mo₂B; Niobium Boride (NbB₂; NbB); Tantalum Boride (TaB₂; TaB); Lanthanum Hexaboride (LaB₆); Barium Hexaboride (BaB₆); Calcium Hexaboride (CaB₆); and Cerium Hexaboride (CeB₆).

The nitrides can include, for example, chemical compositions having the formula MₓN_{y}, where M is a metallic element, N is nitride and X and Y are typically 1. The nitrides have an electrical resistivity in the range of 10⁻⁵ to 10⁻⁴ ohm-cm, and melting points in the range of 1400 to 3300 degrees Celcius. Examples of nitrides include Titanium Nitride (TiN); Zirconium Nitride (ZrN); Tantalum Nitride (TaN); Niobium Nitride (NbN); Vanadium Nitride (VN); and Hafnium Nitride (HfN).

Carbides are another possible ceramic material, including for example chemical compositions having the formula MₓC_{y}, where M is a metallic element, C is carbon and X and Y are typically 1. The carbides typically have an electrical resistivity in the range of 10⁻⁵ to 10⁻⁴ ohm-cm, and melting or sublimation points in the range of 1900 to 4000 degrees Celcius. Some examples include, Tantalum Carbide (TaC); Chromium Carbide (Cr₃C₂); Molybdenum Carbide (MoC; Mo₂C); Tungsten Carbide (WC; W₂C); Zirconium Carbide (ZrC); Titanium Carbide (TiC); Niobium Carbide (NbC); Hafnium Carbide (HfC); Vanadium Carbide (VC); Beryllium Carbide (Be₂C); Silicon Carbide (SiC); and Boron Carbide (B₄C).

The silicides include, for example, chemical compositions having the formula MₓSi_{y}, where M is a metallic element, Si is silicon and X is typically 1 and Y is typically 2. The silicides typically have an electrical resistivity in the range of 10⁻⁵ to 10⁻⁴ ohm-cm, and melting points in the range of 1500 to 2500 degrees Celcius. Some examples include, Molybdenum Silicide (MoSi₂); Niobium Silicide (NbSi₂); Titanium Silicide (TiSi₂); Tungsten Silicide (WSi₂; W₅Si₂); Chromium Silicide (CrSi₂; Cr₃Si); and Tantalum Silicide (TaSi₂).

In another embodiment, the center firing tip **32** is formed of a ceramic material disclosed in U.S. Patent Application No. 12/201,567. In this embodiment, the ceramic material has exceptionally high resistance to high temperature oxidation, erosion and corrosion. The general category of conductive ceramic materials of this embodiment may be referred to as transition metal nitrides, carbides, and carbonitrides due to their superior high temperature properties, including mechanical strength and resistance to certain high temperature oxidation, erosion and corrosion processes. Specifically, the ceramic materials include conductive ceramics of the form Mₙ₊₁AXₙ, where M is a transition metal, A is a group IIIA or IVA element, X is nitrogen, or carbon, or both carbon and nitrogen, and n is 1, 2, or 3. While M may be any transition metal suitable for forming a conductive ceramic compound of the form described above, it is preferred that M be selected from a group consisting of Ti, Nb, Ta, V, Cr, Mo, Sc, Zr and Hf. Even more preferably, M may include Ti, Nb, Ta, V, and Cr, in various combinations. A may be any suitable group IIIA or IVA element or elements, including Al, Ga, In, Tl, Si, Ge, Sn, Pb, P, As and S, with Al and Si believed to be particularly preferred. X may be carbon, nitrogen or both carbon and nitrogen in various stoichiometric and non-stoichiometric proportions.

Exemplary ceramics of this embodiment include Ti₂AlC, Ti₂AlN, Ti₂Al(C0.5, N0.5), Nb₂AlC, (Nb, Ti)AlC, Ti₂AlC, V₂AlC, Cr₂AlC, Ti₄AlN₃, Ti₃AlC2, Ti₂GaC, V₂GaC, Cr₂GaC, Nb₂GaC, Mo₂GaC, Ta₂GaN, Cr₂GaN, Sc₂InC, Ti₂InC, Zr₂InC, Nb₂InC, Hf₂InC, Ti₂InN, Zr₂InN, Ti₂TlC, Zr₂TlC, Hf₂TlC, Zr₂TlN, Ti₃SiC₂, Ti₂GeC, V₂GeC, Cr₂GeC, Ti₃GeC₂, Ti₂SnC, Zr₂SnC, Hf₂SnC, Hf₂SnN, Ti₂PbC, Zr₂PbC, Hf₂PbC, V₂PC, Nb₂PC, V₂AsC, Nb₂AsC, Ti₂SC, Zr₂SC, Nb₂SC, and Hf₂SC. Of these (Nb, Ti)AlC, Ti₂AlC, Va₂AlC, Cr₂AlC, Ti₄AlN₃, Ti₃AlC₂ and Ti₃SiC₂ are believed to be preferred, with Ti₃SiC₂ and Ti₂AlC believed to be particularly preferred.

In another embodiment, the center firing tip **32** is formed of a ceramic material disclosed in U.S. Patent Application No. 12/201,590. In this embodiment, the center firing tip **32** comprises a composite ceramic structure. The composite structure may have at least two different consistent materials, and can either be a ceramic-ceramic composition, or a ceramic-metal (cermet) composition, depending on the specific attributes sought in the specific application. If constructed as a ceramic-ceramic composite, one exemplary composite structure example includes a composite of silicon nitride (Si₃N4) and molybdenum disilicide (MoSi₂).

In one preferred embodiment, the center firing tip **32** is formed of a ceramic-ceramic composite having a uniform composition throughout the firing tip **32.** In alternate embodiment, the concentration of the composition may vary across the width of the center firing tip **32**, in a cross-section taken generally perpendicular to the center axis **A.** Accordingly, the center firing tip **32** of the alternate embodiment has a non-uniform concentration of the different ceramic materials as viewed along a cross-section taken generally perpendicular to the center axis **A.** The difference in composition across the width may provide the center firing tip **32** with an insulating peripheral outer portion and a conductive inner portion surrounded and encapsulated by the outer portion. The inner portion may be exposed or closed along the center firing end **42** and along the center firing surface **36.**

In one exemplary embodiment, without limitation, the composition of the outer portion of the center firing tip **32** can be provided having about 28 percent MoSi₂ and about 72 percent Si₃N₄. The composition of the inner portion can be provided having about 43 percent MoSi₂ and about 57 percent Si₃N₄. Accordingly, the inner portion provides a conductive inner region and the outer portion provides an insulating region. It should be recognized that the aforementioned composite materials are by way of example, and that other materials could be used. For example, the insulating ceramic composite material could be provided as aluminum oxide, aluminum nitride, aluminum oxy-nitride, or silicon aluminum oxynitride, while the conductive ceramic material could be provided as titanium nitride, titanium diboride.

The center firing tip **32** of this embodiment could be provided as a ceramic-metal (cermet) composition, the conductive composite material could be provided as a metal, such as platinum, iridium, nickel or an alloy of nickel, for example. As previously mentioned, the percent concentration of the each of the insulating and conductive ceramic composite materials can be varied across the width of the center firing tip **32** and/or along the length of the center firing tip **32**, depending on the performance requirements desired.

A variety of methods can be used to attach the center firing tip **32** to the center body section. In one embodiment, a braze **50** attaches the center firing tip **32** to the center body portion **28.** The brazing can be done using an active braze alloy, such as Ticusil, Gold-ABA, Gold-ABA-V, or other braze alloys provided by Wesgo Metals. Alternatively, reactive air brazing can be used to attach the center firing tip **32** to the center body portion **28.** The reactive air brazing typically involves using a copper oxide-silver single phase liquid to join the metal of the center body portion **28** and the ceramic material of the center firing tip **32.** The center firing tips **32** of Figures 2-4, 7, 8, 10, and 11 may be attached by brazing.

In another embodiment, the center electrode **22** includes a retaining element **52** disposed along the center firing end **42** for attaching the center firing tip **32** to the center body portion **28.** In one embodiment, as shown in Figures 5 and 6, the retaining element **52** includes a ledge or other mechanical locking feature facing inwardly toward the center axis **A.** The retaining element **52** and center firing end **42** together present the center hole **48** therebetween for receiving the center firing tip **32** and mechanically attaching the center firing tip **32** to the center body portion **28.** In the embodiment of Figure 6, the retaining element **52** is attached to the center body portion **28** by a laser weld **86.** In yet another embodiment, as shown in Figure 9, the center firing tip **32** is attached to the center body portion **28** by forming indentations **82**, holes, grooves, or notches along the center firing tip **32** adjacent the center firing end **42**, and melting a portion of the center body portion **28** at the center firing end **42**, adjacent the indentations, so that the body portion **28** flows into the indentations and solidifies, providing the melted portion **88** of Figure 9. The melted portion **88** secures the center firing tip **32** to the center body portion **28.**

As shown in Figure 1, the spark plug **20** further includes other elements such as those typically found in spark plugs **20** of internal combustion engines. For example, the spark plug **20** includes an insulator **56** disposed annularly around the center electrode **22.** The insulator **56** extends longitudinally from an insulator upper end **58**, along the center body portion **28**, toward the center firing end **42**, and to an insulator firing end **60.** The center firing end **42** projects outwardly of the insulator firing end **60.**

The insulator **56** is formed of an electrically insulating material, such as alumina. The insulator **56** preferably has a very low dielectric loss factor, and an electrical conductivity significantly less than the electrical conductivity of the center electrode 22, such as an electrical conductivity of not greater than 10⁻¹² S/m.

The spark plug **20** of Figure 1 includes a terminal **62** formed of an electrically conductive material received in the insulator **56** and extending from a first terminal end **64** to a second terminal end **66**, which is electrically connected to the center electrode top end **40** of the center electrode **22.** The terminal **62** is formed of an electrically conductive material. A resistor layer **68** is disposed between and electrically connects the second terminal end **66** of the terminal **62** and the center electrode top end **40** of the center electrode **22** for transmitting energy from the terminal **62** to the center electrode **22.** The resistor layer **68** is formed of an electrically resistive material, such as a glass seal.

The spark plug **20** further includes a shell **70** disposed annularly around and longitudinal along the insulator **56** from an upper shell end **72** to a lower shell end **74.** The insulator firing end **60** and the center firing end **42** project outwardly of the lower shell end **74**, as shown in Figure 1. The spark plug **20** engages with the engine by means of a threaded portion of the shell **70**, where the threads **84** may be 14 mm, 12 mm, or 10 mm, and preferably 12 mm. However, it will be understood by those of ordinary skill in the art that other threads, or other means of engaging with the engine, can be used. The shell **70** is formed of a metal material, such as steel. The spark plug **20** can include at least one packing element **54**, such a gasket, cement, or other sealing compound, disposed between the insulator **56** and the shell **70** for providing a gas-tight seal between the shell **70** and the insulator **56.** The packing element **54** can also be disposed between the insulator **56** and the terminal **62.**

The ground electrode **24** of the spark plug **20** is attached to the lower shell end **74** of the shell **70.** The ground electrode **24** comprises the body portion **30**, referred to as a ground body portion **30**, extending from a ground electrode top end **76**, which is attached to the lower shell end **74**, to a ground firing end **78.** The ground body portion **30** extends transversely from the lower shell end **74** and curves toward the center electrode **22** to the ground firing end **78.**

Like the center body portion **28** of the center electrode **22**, the ground body portion **30** also includes a thermally conductive material, which is typically selected from the same group of materials as the thermally conductive material of the center body portion **28**, but can be a different material. In one embodiment, the ground body portion **30** includes the clad **44** of the thermally conductive material, such as nickel, enrobing the core **46** of another thermally conductive material, such as copper. The ground body portion **30** has a thermal conductivity sufficient to draw heat away from a ceramic ground firing tip **34.** The ground body portion **30** has a thermal conductivity of at least 20 Wm-K when measured at 20° C, and preferably at least 35 W/m-K when measured at 20° C.

The ground body portion **30** also has an electrical conductivity of at least 9 x 10⁵ S/m. As shown in Figure 1, the ground body portion **30** has a first length **l₁** extending parallel to the center axis **A.** In one embodiment (not shown), the ground body portion **30** includes a clad of a first thermally conductive material, such as nickel, and a core of a second thermally conductive material, such as copper, enrobed by the clad. The thermally conductive material of the core is also electrically conductive.

As alluded to above, the ground electrode **24** preferably includes a firing tip **34**, referred to as the ground firing tip **34**, extending transversely from the ground firing end **78** toward the center firing tip **32.** The ground firing tip **34** has a second length **l₂** extending parallel to the center axis **A**, which is generally less than the first length **l₁**, but may be longer than the first length **l₁.** The ground firing tip **34** also preferably includes one of the ceramic materials described above with regard to the center firing tip **32.** The ceramic material of the ground firing tip **34** can be the same as or different from the ceramic material of the center firing tip **32.** The ceramic material of the ground firing tip **34** provides the firing surface **36, 38**, referred to as a ground firing surface **38**, facing the center firing surface **36** and exposed to the combustion chamber.

As shown in Figures 1 and 1A, the ground firing surface **38** is spaced and parallel to the center firing surface **36** to provide the spark gap **26** therebetween. However, in an alternate embodiment, only one of the electrodes **22, 24** includes the firing tip **32, 34,** and the spark gap **26** is provided in part by another type firing surface of the electrode **22, 24** without the firing tip **32, 34.** In one embodiment, the ground firing tip **34** has a rectangular cross-section, but can comprise a variety of shapes, being the same as or different from the center firing tip **32.** The ground firing tip **34** can be attached to the ground body portion **30** by a variety of methods, such as those discussed with regard to the center firing tip **32** and the center body portion **28.** In one embodiment, the ground body portion **30** presents a ground hole **80** extending longitudinally along the center axis **A** and facing outwardly of the ground electrode **24** at the ground firing end **78.**

In one embodiment, the ground firing tip **34** of the ground electrode **24** is constructed of at least one oxide. For example, 100 weight percent (wt. %) of the ground firing tip **34** could consist of the at least one oxide. Alternatively, at least 50 wt. %, or at least 70 wt. %, or at least 90 wt. %, or at least 95 wt. % of the ground firing tip **34** could consist of the at least one oxide. The at least one oxide used to form the ground firing tip **34** typically includes oxides of transition metals. In this embodiment, the oxides can include monoxides, such as TiO, VO, NbO, TaO, MnO, FeO, CoO, NiO, CuO, and ZnO; sesquioxides, such as V₂O₃, CrO₃, Fe₂O₃, RhO₃, In₂O₃, Th₂O₃, and Ga₂O₃; and dioxides such as TiO₂, VO₂, CrO₂, MoO₂, WO₂, RuO₂, ReO₂, OsO₂, RhO₂, IrO₂, PbO₂, NbO₂, MbO₂, MnO₂, PtO₂, GeO₂, and SnO₂.

The at least one oxide of the ground firing tip **34** can also include oxides of two or more metals, which include at least one transition metal. Such oxides include perovskite structures with the general formulation ABO₃, wherein component A includes at least one of La, Ca, Ba, Sr, Y, and Gd; and component B includes at least one of Sc, Ti, Zr, Hf, Nb, Ta, Mo, W, Re, V, Cr, Mn, Tc, Fe, Ru, Co, Rh, Ga, and Ni. Examples of such perovskite structures include LaCrO₃, LaMnO₃, LaFeO₃, LaGaO₃, and LaCoO₃.

In another embodiment, at least a portion of the component A and/or at least a portion of the component B of the perovskite structure can be replaced or substituted with a another component C and/or component D. In other words, some of component A, or all of component A, could be replaced with component C and/or component D; and some of component B, or all of component B, could be replaced with component C and/or component D. In an exemplary embodiment, component C includes at least one of La, Ca, Ba, Sr, Y, and Gd; and is different from component A and B. Component D includes at least one of Sc, Ti, Zr, Hf, Nb, Ta, Mo, W, Re, V, Cr, Mn, Tc, Fe, Ru, Co, Rh, and Ni; and is different from component A and B. For example, the perovskite structure with the formulation ABO₃ could be substituted with the additional component C and/or component D to form a perovskite with the general formulation (AₓC₁₋ₓ)BO₃, A(B_{y}D_{1-y})O₃ or (AₓB₁₋ₓ)(C_{y}D_{1-y})O₃, wherein x is between 0 and 0.5 and y is between 0 and 0.5. A specific example of the alternate perovskite structure is La₁₋ₓSrₓMnO₃, wherein a portion of the La is substituted with Sr. In addition, in certain embodiments, there could be three or more elements that occupy component A, which are each selected from the list of component A above; and/or three or more elements that occupy component B, which are each selected from the list of component B above.

Furthermore, components C and D may include elements selected from a group that have a valence charge different from that of components A and/or B, so that the total amount of oxygen (O) can be greater than or less than 3. For example, the alternate perovskite structure could have the general formulation MₓN_{1-y}O_{3-z}, wherein component M comprises component A and at least one other metallic element; component N comprises component B and at least one other metallic element; x is in the range from 0.9 to 1.1; y is in the range from 0.9 to 1.1; and z is in the range from -0.2 to 0.2. In an exemplary embodiment, the at least one other metallic element of component M and/or component N is selected from the following group: La, Ca, Ba, Sr, Y, Gd, Sc, Ti, Zr, Hf, Nb, Ta, Mo, W, Re, V, Cr, Mn, Tc, Fe, Ru, Co, Rh, Ni, Cu, Zn, Ag, Ga, Al, and Si. In this embodiment, the valence charge of the other metallic element of component M is different than the valence charge of component A, and the valence charge of the other metallic element of component N is different from the valence charge of component B.

The at least one oxide used to construct the ground firing tip **34** of the ground electrode **24** could alternatively comprise a spinel structure having the general formulation AB₂O₄, wherein component A includes at least one of Li, Co, Mg, Zn, Ni, Fe, Cd, Mn, and Cu; and component B includes at least one of Al, Cr, and Fe. An exemplary spinel structure is nickel ferrite, which is an electrically conducting spinel having the stoichiometric composition NiFe₂O₄. In one embodiment, the performance of the spinel is improved by changing the ratio of Ni and Fe, such that the general formulation of the spinel is Ni₁₋ₓFe₂₊ₓO₄ or Ni₁₊ₓFe₂₋ₓO₄, wherein x ranges from 0 to 0.5.

In another embodiment, at least a portion of the component A and/or at least a portion of the component B of the spinel structure can be replaced with another component C and/or component D. In other words, some of component A, or all of component A, could be replaced with component C and/or component D; and some or component B, or all of component B, could be replaced with component C and/or component D. In an exemplary embodiment, component C includes at least one of Li, Co, Mg, Zn, Ni, Fe, Cd, Mn, Cu, Mo, W, Cr and V; and component C is different from component A and B. Component D includes at least one of Al, Cr, Fe, Co, Ga and Mo; and component D is different from component A and B. Like the perovskite structures, the spinels can be substituted, in which case the general formulation would be MₓN_{2-y}O_{4-z}, wherein M comprises component A and at least one other metallic element; N comprises component B and at least one other metallic element; x ranges from -0.1 to 0.1; y ranges from -0.1 to 0.1; and z ranges from -0.2 to 0.2. In an exemplary embodiment, the at least one other metallic element of component M and/or component N is selected from the following group: Ge, V, Te, Ti, Sb, Nb, Ta, W, Sn, Hf, Zr, Sc, Bi, and In.

The ground firing tip **34** constructed of the perovskite structure or spinel structure is manufactured by compacting and sintering the ceramic material. In one embodiment, the ceramic material initially provided for compacting and sintering includes at least one of the perovskite structures or spinel structures described above.

In another embodiment, a precursor material is provided which upon sintering forms one of the perovskite structures or spinel structures. The precursor material typically includes common oxides and/or carbonates of the elements listed above. Exemplary precursor materials that can be compacted and sintered to form the ground firing tip **34** from a perovskite structure include at least one of La₂O₃, CaCO₃, BaCO₃, SrCO₃, Y₂O₃, Gd₂O₃, Sc₂O₃, TiO₂, ZrO₂, HfO₂, Nb₂O₅, Ta₂O₅, MoO₃, MO₂O₃, WO₃, ReO₃, V₂O₃, Cr₂O₃, MnO₂, Fe₂O₃, FeO, Fe₃O₄, RuO₄, CoO, NiO, and Ni₂O₃. Exemplary precursor materials that can be compacted and sintered to form the ground firing tip **34** from a spinel structure include at least one of Li₂CO₃, CoO, MgCO₃, MgO, ZnO, NiO, Ni₂O₃, FeO, Fe₂O₃, Fe₃O₄, CdO, MnO₂, CuO, Al₂O₃, Al(OH)₃ and Cr₂O₃.

Another aspect of the invention provides a method of forming the spark plug **20** described above. The method includes providing the electrode **22, 24** by compacting the ceramic material to form the firing tip **32, 34**; sintering the compacted ceramic material; and disposing the firing tip **32, 34** on the body portion **28, 30**, either before or after sintering. The method can include disposing the ceramic firing tip **32, 34** on the center electrode **22**, the ground electrode **24**, or both. In one embodiment, the method includes forming a hole **48, 80** along the center axis **A**, and disposing the firing tip **32, 34** in the hole **48, 80.**

In another embodiment, the method of forming the spark plug **20** includes brazing the firing tip **32, 34** to the body portion **28, 30.** As stated above, the brazing step can include using an active braze alloy, such as Ticusil, Gold-ABA, Gold-ABA-V, or other braze alloys provided by Wesgo Metals. Alternatively, the brazing can include reactive air brazing, which typically involves using a copper oxide-silver single phase liquid to join the metal of the body portion **28, 30** and the ceramic material of the firing tip **32, 34.**

Alternatively, the method can include mechanically attaching the firing tip **32, 34** to the body portion **28, 30.** A retaining element **52** can be used to attach the firing tip **32, 34** to the body portion **28, 30.** In one embodiment, the method includes brazing or laser welding the retaining element **52** to the body portion **28, 30.** In yet another embodiment, the firing tip **32, 34** is attached to the body portion **28, 30** by forming indentations **82,** holes, grooves, or notches along sides of the firing tip **32, 34** adjacent the body portion **28, 30,** heating, and melting a portion of the body portion **28, 30** at the firing end **42, 78** adjacent the holes. The body portion **28, 30** flows into the holes and solidifies, providing the melted portion **88** of Figure 9, securing the firing tip **32, 34** to the body portion **28, 30.**

In one exemplary embodiment, the method first comprises compacting the ceramic material to form the firing tip **32, 34**, wherein the ceramic material includes at least one of a perovskite structure, a spinel structure, and a precursor material that forms a perovskite or spinel structure upon sintering. The method further includes sintering the compacted ceramic material; and disposing the sintered ceramic material on the body portion **28, 30** including a thermally conductive material, either before or after the sintering step.

Obviously, many modifications and variations of the present invention are possible in light of the above teachings and may be practiced otherwise than as specifically described while within the scope of the appended claims. These antecedent recitations should be interpreted to cover any combination in which the inventive novelty exercises its utility. In addition, the reference numerals in the claims are merely for convenience and are not to be read in any way as limiting.

## Claims

1. A spark plug (20) for igniting a mixture of fuel and air of an internal combustion engine, comprising:
an electrode (22, 24) having a body portion including a thermally conductive material;
said electrode (22, 24) having a firing tip (32, 34) disposed on said body portion (28, 30);
said firing tip (32, 34) including a ceramic material, and said ceramic material including at least one perovskite structure,
wherein the at least one perovskite structure includes the formulation ABO₃, wherein component A includes at least one of La, Ca, Ba, Sr, Y, and Gd; component B includes at least one of Sc, Ti, Zr, Hf, Nb, Ta, Mo, W, Re, V, Cr, Mn, Tc, Fe, Ru, Co, Rh, Ga, and Ni; and at least a portion of component A and/or at least a portion of component B of the perovskite structure is replaced with component C and/or component D, wherein component C is different from components A and B and includes at least one of La, Ca, Ba, Sr, Y, and Gd; and component D is different from components A and B and includes at least one of Sc, Ti, Zr, Hf, Nb, Ta, Mo, W, Re, V, Cr, Mn, Tc, Fe, Ru, Co, Rh, Ga, and Ni.

2. The spark plug (20) of claim 1, wherein at least 50 wt. % of said firing tip (32, 34) consists of the at least one perovskite structure.

3. The spark plug (20) of claim 1, wherein the at least one perovskite structure includes one of the following formulations: (AₓC₁₋ₓ)BO₃, A(B_{y}D_{1-y})O₃, or (AₓB₁₋ₓ)(C_{y}D_{1-y})O₃; wherein component A includes at least one of La, Ca, Ba, Sr, Y, and Gd; component B includes at least one of Sc, Ti, Zr, Hf, Nb, Ta, Mo, W, Re, V, Cr, Mn, Tc, Fe, Ru, Co, Rh, Ga, and Ni; x is between 0 and 0.5; and y is between 0 and 0.5.

4. The spark plug (20) of claim 3, wherein the at least one perovskite structure includes La₁₋ₓSrₓMnO₃.

5. The spark plug (20) of claim 1, wherein the at least one perovskite structure includes the formulation MₓN_{1-y}O_{3-z}, wherein component M comprises component A and at least one other metallic element; component A includes at least one of La, Ca, Ba, Sr, Y, and Gd; component N comprises component B and at least one other metallic element; component B includes at least one of Sc, Ti, Zr, Hf, Nb, Ta, Mo, W, Re, V, Cr, Mn, Tc, Fe, Ru, Co, Rh, Ga, and Ni; x ranges from 0.9 to 1.1; y ranges from 0.9 to 1.1; and z ranges from -0.2 to 0.2.

6. The spark plug (20) of claim 5, wherein the at least one other metallic element of component M includes at least one of La, Ca, Ba, Sr, Y, Gd, Sc, Ti, Zr, Hf, Nb, Ta, Mo, W, Re, V, Cr, Mn, Tc, Fe, Ru, Co, Rh, Ni, Cu, Zn, Ag, Ga, Al, and Si; and the at least one other metallic element of component N includes at least one of La, Ca, Ba, Sr, Y, Gd, Sc, Ti, Zr, Hf, Nb, Ta, Mo, W, Re, V, Cr, Mn, Tc, Fe, Ru, Co, Rh, Ni, Cu, Zn, Ag, Ga, Al, and Si.

7. The spark plug (20) of claim 6, wherein the at least one other metallic element of component M has a valence charge different from the valence charge of component A; and the at least one other metallic element of component N has a valence charge different from the valence charge of component B.

8. A spark plug (20) for igniting a mixture of fuel and air of an internal combustion engine, comprising:
an electrode (22, 24) having a body portion (28, 30) including a thermally conductive material;
said electrode (22, 24) having a firing tip (32, 34) disposed on said body portion (28, 30);
said firing tip (32, 34) including a ceramic material, and said ceramic material including at least one spinel structure,
wherein the spinel structure has the formulation AB₂O₄, wherein component A includes at least one of Li, Co, Mg, Zn, Ni, Fe, Cd, Mn, and Cu; component B includes at least one of Al, Cr, and Fe; and at least a portion of component A and/or at least a portion of component B is replaced with component C and/or component D; wherein component C is different from component A and B and includes at least one of Li, Co, Mg, Zn, Ni, Fe, Cd, Mn, Cu, Mo, W, Cr and V; and component D is different from component A and B and includes at least one of Al, Cr, Fe, Co, Ga and Mo..

9. The spark plug (20) of claim 8, wherein at least 50 wt. % of said firing tip consists of the at least one spinel structure.

10. The spark plug (20) of claim 8, wherein the spinel structure is nickel ferrite having the formulation Ni₁₋ₓFe₂₊ₓO₄ or Ni₁₊ₓFe₂₋ₓO₄; and x ranges from 0 to 0.5.

11. The spark plug (20) of claim 10, wherein the nickel ferrite has the formulation NiFe₂O₄.

12. The spark plug (20) of claim 8, wherein the spinel structure has the formulation MₓN_{2-y}O_{4-z}, wherein component M comprises component A and at least one other metallic element; component N comprises component B and at least one other metallic element; x ranges from -0.1 to 0.1; y ranges from -0.1 to 0.1; and z ranges from -0.2 to 0.2.

13. The spark plug (20) of claim 12, wherein the at least one other metallic element of M is selected from the following group: Ge, V, Te, Ti, Sb, Nb, Ta, W, Sn, Hf, Zr, Sc, Bi, and In; and the at least one other metallic element of N is selected from the following group: Ge, V, Te, Ti, Sb, Nb, Ta, W, Sn, Hf, Zr, Sc, Bi, and In.

14. An electrode (22, 24) for an ignition device (20), comprising:
a body portion (28, 30) including a thermally conductive material;
a firing tip (32, 34) disposed on said body portion (28, 30);
said firing tip (32, 34) including a ceramic material, and said ceramic material including at least one of a perovskite structure and a spinel structure,
wherein the perovskite structure includes the formulation ABO₃, wherein component A includes at least one of La, Ca, Ba, Sr, Y, and Gd; component B includes at least one of Sc, Ti, Zr, Hf, Nb, Ta, Mo, W, Re, V, Cr, Mn, Tc, Fe, Ru, Co, Rh, Ga, and Ni; and at least a portion of component A and/or at least a portion of component B of the perovskite structure is replaced with component C and/or component D, wherein component C is different from components A and B and includes at least one of La, Ca, Ba, Sr, Y, and Gd; and component D is different from components A and B and includes at least one of Sc, Ti, Zr, Hf, Nb, Ta, Mo, W, Re, V, Cr, Mn, Tc, Fe, Ru, Co, Rh, Ga, and Ni., wherein at least a portion of component A and/or at least a portion of component B of the perovskite structure is replaced with component C and/or component D,
and wherein the spinel structure has the formulation AB₂O₄, wherein component A includes at least one of Li, Co, Mg, Zn, Ni, Fe, Cd, Mn, and Cu; component B includes at least one of Al, Cr, and Fe; and at least a portion of component A and/or at least a portion of component B is replaced with component C and/or component D; wherein component C is different from component A and B and includes at least one of Li, Co, Mg, Zn, Ni, Fe, Cd, Mn, Cu, Mo, W, Cr and V; and component D is different from component A and B and includes at least one of Al, Cr, Fe, Co, Ga and Mo.

15. A method of manufacturing an electrode (22, 24) for an ignition device (20), comprising the steps of:
compacting a ceramic material to form a firing tip, wherein the ceramic material includes at least one of a perovskite structure, a spinel structure, and a precursor material that forms a perovskite or spinel structure upon sintering;
sintering the compacted ceramic material; and
disposing the sintered ceramic material on a body portion including a thermally conductive material,
wherein the perovskite structure includes the formulation ABO₃, wherein component A includes at least one of La, Ca, Ba, Sr, Y, and Gd; component B includes at least one of Sc, Ti, Zr, Hf, Nb, Ta, Mo, W, Re, V, Cr, Mn, Tc, Fe, Ru, Co, Rh, Ga, and Ni; and at least a portion of component A and/or at least a portion of component B of the perovskite structure is replaced with component C and/or component D, wherein component C is different from components A and B and includes at least one of La, Ca, Ba, Sr, Y, and Gd; and component D is different from components A and B and includes at least one of Sc, Ti, Zr, Hf, Nb, Ta, Mo, W, Re, V, Cr, Mn, Tc, Fe, Ru, Co, Rh, Ga, and Ni., wherein at least a portion of component A and/or at least a portion of component B of the perovskite structure is replaced with component C and/or component D,
and wherein the spinel structure has the formulation AB₂O₄, wherein component A includes at least one of Li, Co, Mg, Zn, Ni, Fe, Cd, Mn, and Cu; component B includes at least one of Al, Cr, and Fe; and at least a portion of component A and/or at least a portion of component B is replaced with component C and/or component D; wherein component C is different from component A and B and includes at least one of Li, Co, Mg, Zn, Ni, Fe, Cd, Mn, Cu, Mo, W, Cr and V; and component D is different from component A and B and includes at least one of Al, Cr, Fe, Co, Ga and Mo.
